

# United States Patent [19]

Niimi et al.

[11] 3,928,241

[45] Dec. 23, 1975

[54] CATALYSTS FOR PURIFYING EXHAUST GAS

|           |         |                          |             |
|-----------|---------|--------------------------|-------------|
| 3,206,414 | 9/1965  | Gunther .....            | 252/474     |
| 3,565,574 | 2/1971  | Kearby et al. ....       | 252/474 X   |
| 3,699,683 | 10/1972 | Tourtellotte et al. .... | 423/213.2 X |
| 3,718,733 | 2/1973  | Gehri .....              | 423/213.2   |
| 3,773,894 | 11/1973 | Bernstein et al. ....    | 252/474 X   |

[75] Inventors: **Itaru Niimi**, Nagoya; **Yasuhide Kaneko**, Toyota; **Akiyoshi Morita**, Toyota; **Yasuo Nemoto**, Toyota; **Mitsuyoshi Sato**, Toyota, all of Japan

[73] Assignee: **Toyota Jidosha Kogyo Kabushiki Kaisha**, Japan

[22] Filed: **Feb. 12, 1973**

[21] Appl. No.: **331,888**

[30] Foreign Application Priority Data

Feb. 12, 1972 Japan..... 47-14983

[52] U.S. Cl. .... **252/470; 252/474; 423/213.5**

[51] Int. Cl. .... **B01J 23/86; B01J 23/72**

[58] Field of Search ..... 252/470, 474; 423/213.2, 423/213.5, 213.7

[56] References Cited

UNITED STATES PATENTS

2,564,844 8/1951 Hodge..... 252/470 X

FOREIGN PATENTS OR APPLICATIONS

|         |        |                     |           |
|---------|--------|---------------------|-----------|
| 354,692 | 2/1930 | United Kingdom..... | 423/213.2 |
|---------|--------|---------------------|-----------|

Primary Examiner—W. J. Shine  
Attorney, Agent, or Firm—Connolly and Hutz

[57] ABSTRACT

Exhaust gas purifying catalysts characterized in that alloys comprising 0.1-40% of Cu and the balance of Ni and/or Fe by weight as fundamental components are shaped as desired and are activated, at least partially, by providing their surfaces with oxidized enriched Cu layers thicker than  $10\mu$  in the oxidization atmosphere or by partially reducing the oxidized layers with hydrogen gas at high temperature.

3 Claims, 16 Drawing Figures

*Fig. 1.*



Fig. 2.



*Fig. 3a.*



Casted as is  
Fe-2.8%Ni-0.5%Cu  
(Specimen No. 1)

*Fig. 3b.*



After annealing  
X 200

*Fig. 4a.*



Casted as is  
Fe-2.5%Cu  
(Specimen No. 16)

*Fig. 4b.*



After annealing  
X 200

*Fig. 5.*



Ni-24.0%Cu  
(Specimen No. 18)  
X 200

*Fig. 6a.*

Casted as is  
Fe-32.0%Ni-17.7%Cu-3.9%Al  
(Specimen No. 27)

*Fig. 6b.*

After annealing  
X 200

*Fig. 7.**Fig. 8a.*

Casted as is  
X 200  
Fe-47.6%Ni-17.7%Cu  
-1.5%C-1.6%Si  
(Specimen No. 22)

*Fig. 8b.*

Casted as is  
Fe-28.9%Cu-33.0%Co  
(Specimen No. 33)



After annealing  
X 200

*Fig. 9.*

X 1000  
Surface of alloy  
without oxidized layer

*Fig. 10a.*

X 300  
Fe-52.0%Ni-26.4%Cu  
(Oxidized layer thickness 0.6mm  
Oxidized at 900°C. for 24 hours)

*Fig. 10b.*

X 1000  
Fe-52.0%Ni-26.4%Cu  
(Oxidized layer thickness 0.6mm  
Oxidized at 900°C. for 24 hours)

*Fig. 10c.*

X 3000  
Fe-52.0%Ni-26.4%Cu  
(Oxidized layer thickness 0.6mm  
Oxidized at 900°C for 24 hours)

## CATALYSTS FOR PURIFYING EXHAUST GAS

### BACKGROUND OF THE INVENTION

The present invention relates to a catalyst for purifying exhaust gas.

Conventional industrial catalysts suitable for purifying exhaust gas are agents which are generally made by allowing carriers such as alumina to carry noble metals such as Pt or Pd or carry or mix with oxides of Ni, Cu or Cr. But these are significantly disadvantageous in that catalytic agents comprising noble metals such as Pt or Pd are expensive, their resources are insufficiently available, inferiority in heat resistance and durability, and unsuitability for quantity production due to difficult manufacturing methods. Various other alloy system catalysts are known in addition to catalysts as mentioned above, but these do not demonstrate their effects if temperature is not high.

### SUMMARY OF THE INVENTION

Accordingly, it is an object of the present invention to provide a unique catalyst for purifying exhaust gas which avoids the drawbacks of the prior art and which functions in a highly beneficial and economical manner.

The present invention relates to exhaust gas purifying catalysts having characteristics for removing harmful nitrogen oxide (NO<sub>x</sub>) components contained in exhaust gases, particularly those from internal combustion engines, by reduction, and is characterized in that alloys comprising 0.1 - 40% of Cu and the balance of Ni and/or Fe by weight are provided with enriched Cu layers on their surface portions, or further, the oxidized layers are partially activated.

### BRIEF DESCRIPTION OF THE DRAWINGS

Novel features and advantages of the present invention in addition to those mentioned above will become apparent to those skilled in the art from a reading of the following detailed description in conjunction with the accompanying drawings wherein similar reference characters refer to similar parts and in which:

FIG. 1 is a diagram of alloy composition ranges of the catalysts according to the present invention;

FIG. 2 is a graph diagram showing the relationship between NO and CO purification rates and catalyst bed temperatures;

FIG. 3 through 8 are microscopic photographs of typical alloys and catalysts obtained in embodying Examples 1 through 6 according to the present invention;

FIG. 9 is a photograph made by a scanning-type electronic microscope illustrating the state of an alloy surface in the case where an oxidized layer is absent from the surface; and

FIG. 10 comprises photographs made by a scanning-type electronic microscope illustrating the state of an alloy surface in the case where an oxidized layer thicker than 10 $\mu$  is present.

### DETAILED DESCRIPTION OF THE INVENTION

The present invention is intended to provide catalysts for reducing and removing NO<sub>x</sub> contained in exhaust gas discharged from internal combustion engines. The catalysts achieve remarkable effects for removing harmful components under comparatively low temperatures ranging from 400° to 600°C., allow wider alloy selective range and can selectively formed in accor-

dance with a wide range of applications. Compositions and manufacturing of exhaust gas purifying catalysts according to the present invention are described below.

As for compositions of alloys according to the present invention, catalysts of this invention comprise a binary Fe-Cu or Ni-Cu or a ternary Fe-Ni-Cu system alloy (hereinafter referred to as this system's alloy) always containing less than 99.9% of Fe and Ni and the balance of Cu.

In this case, it is possible to reduce contents of Fe and Ni as desired and instead, to add elements other than Fe, Ni and Cu less than 10% by weight.

The type of elements to be added is not particularly restricted, but since Co and Cr efficiently achieve the catalytic effect, addition of those elements up to 40% by weight is acceptable. Co demonstrates the effect similar to that of Cu. Of course, nonmetallic elements such as C and Si which are contained in usual alloys also may be added.

20 A composition range of this system's alloy for the catalysts according to the present invention is given in FIG. 1. A portion rectangularly surrounded by ABCD is a standard composition range. Even in case other additive elements are contained, if the composition rate is within a diagonally lined range, that composition is acceptable.

In the present invention, this system's alloy within the above composition range is obtained by the conventional method and is shaped in workable plasticity types such as a sheet, bar, pipe, line or alloy powder, casting materials, etc., according to alloy compositions and applications for use as catalysts.

It is an essential factor in producing alloy catalysts to place oxidized layers thicker than 10 $\mu$  over the alloys.

35 The catalysts according to the present invention, can function satisfactory with an oxidized layer only, but those are further improved by reducing the oxidized layers formed on alloys. Descriptions as to examples embodying the present invention are given below. In each of these examples only one-half of the specimen is reduced after oxidation to thereby provide a comparison between oxidation alone and reduction after oxidation.

### EXAMPLE 1

After melting Fe-Ni-Cu ternary alloys with various compositions as given in Table 1 at 1600°C. by using a Tammann furnace, a casting was made in a stainless steel (SUS 27) mold coated with a sufficient thickness of graphite. After casting, casted cylindrical bars obtained were machined to make cuttings and were subjected to oxidation treatment in a high temperature atmosphere at 1000°C. for six hours to obtain catalyst cuttings.

55 By producing the cuttings as described above, an apparent surface area per unit weight becomes wider. The dimensions of the cuttings vary with the material, but those within the range of 0.1 - 0.5mm in thickness, 2mm-20mm in length and 1mm-3mm in width are desirable. The term "Cuttings" in this Example and hereinafter, represents granularity almost within the above range.

Further, half of the catalyst (after oxidation) obtained as above, was reduced at 800°C. in hydrogen gas for two hours. Alloy compositions and purification rates of the catalyst obtained by the above process are given in Table 1. Chemical components given in the Table show alloy compositions after casting and the

purification rates are results of the test using 10ml of the catalyst. The above explanations are common in Table 2 and succeeding tables.

The catalyst's apparent surface area of 10ml is dependent on the catalyst components, but is almost within 100 – 1000cm<sup>2</sup>. Unless otherwise specified, the surface area is identical to that in Example 1.

### EXAMPLE 2

The binary alloy with a composition of Fe and Cu as given in Table 2 was casted at 1650°C. in the same metal mold as in Example 1 after being melted in a high frequency furnace.

Casted cylindrical bars obtained were machined to make cuttings and the cuttings were subjected to oxidation treatment in an atmosphere at 1100°C. for three hours to obtain catalysts. Also, half of the cuttings were reduced in hydrogen gas at 800°C. for two hours to obtain catalysts.

### EXAMPLE 3

A sheet-type catalyst was obtained by subjecting 0.5mm thickness of an Ni-Cu alloy to atmospheric oxidation at 800°C., 900°C., 1000°C. and 1100°C. for 24, 12, 6 and 3 hours, respectively.

This sheet-type catalyst had been shaped cylindrically at 0.5mm in thickness, 2.5mm in width and 15mm in length. A half of the catalyst was subjected to hydrogen gas reduction at 800°C. for 2 hours. Apparent surface area of a 10ml catalyst obtained by the above process was approximately 100cm<sup>2</sup>.

### EXAMPLE 4

Fe-Ni-Cu alloy comprising other additive elements as given in Table 4 was made into cuttings and subjected to high temperature atmospheric oxidation at 1000°C. for 6 hours, and a half was subjected to hydrogen gas reduction at 800°C. for 2 hours.

### EXAMPLE 5

Fe-Cu binary alloy comprising other additive elements as given in Table 5 was made into cuttings and subjected to high temperature atmospheric oxidation at 1100°C. for three hours, and a half was subjected to hydrogen gas reduction at 800°C. for 2 hours.

### EXAMPLE 6

Ni-Cu alloy comprising other additive elements as given in Table 6 was formed into a 1.0mm thick sheet and subjected to high temperature atmospheric oxidation at 900°C. for twelve hours to obtain a sheet-type catalyst, and a half was subjected to hydrogen gas reduction at 800°C. for 2 hours. The sheet with dimensions of 1.0mm × 2.5mm × 15mm, the same as in Example 3, was cylindrically formed. Apparent surface area of 10ml catalyst was approximately 100cm<sup>2</sup>.

Table 1

| Specimen No. | Chemical component (%) |      |     | Compositions and purification rates of Fe-Ni-Cu system alloys |                     |
|--------------|------------------------|------|-----|---------------------------------------------------------------|---------------------|
|              | Cu                     | Ni   | Fe  | NO purification rate                                          | Oxidation/Reduction |
|              |                        |      |     | Oxidation                                                     |                     |
| 1            | 0.5                    | 2.8  | bal | 30.0                                                          | 68.2                |
| 2            | 0.8                    | 3.6  | bal | 53.4                                                          | 74.5                |
| 3            | 0.9                    | 8.9  | bal | 28.4                                                          | 56.1                |
| 4            | 1.8                    | 9.1  | bal | 56.0                                                          | 36.2                |
| 5            | 2.6                    | 8.7  | bal | 19.5                                                          | 64.3                |
| 6            | 4.4                    | 50.8 | bal | 51.3                                                          | 86.2                |
| 7            | 5.2                    | 9.5  | bal | 30.7                                                          | 49.9                |
| 8            | 5.3                    | 20.3 | bal | 4.0                                                           | 58.1                |
| 9            | 6.4                    | 17.5 | bal | 3.3                                                           | 80.0                |
| 10           | 7.4                    | 9.9  | bal | 4.3                                                           | 53.2                |
| 11           | 8.8                    | 35.4 | bal | 6.6                                                           | 57.8                |
| 12           | 9.5                    | 15.0 | bal | 4.0                                                           | 74.3                |
| 13           | 10.9                   | 42.1 | bal | 0                                                             | 72.1                |
| 14           | 18.1                   | 22.3 | bal | 0                                                             | 70.8                |
| 15           | 26.4                   | 52.0 | bal | 0                                                             | 78.5                |

Table 2

| Specimen No. | Chemical component (%) |     |  | Compositions and purification rates of Fe-Cu system alloys |                      |
|--------------|------------------------|-----|--|------------------------------------------------------------|----------------------|
|              | Cu                     | Fe  |  | Oxidation/Reduction                                        | NO purification rate |
|              |                        |     |  | Oxidation                                                  |                      |
| 16           | 2.5                    | bal |  | Oxidation                                                  | 6.8                  |
| 17           | 4.6                    | bal |  | Reduction after oxidation                                  | 70.0                 |
|              |                        |     |  | "                                                          | 8.0                  |
|              |                        |     |  | "                                                          | 71.8                 |

Table 3

| Specimen No. | Chemical component (%) |    |  | Treatment conditions and purification rates of Ni-Cu alloys |                          |                          |
|--------------|------------------------|----|--|-------------------------------------------------------------|--------------------------|--------------------------|
|              | Cu                     | Ni |  | Oxidation/Reduction                                         | NO purification rate (%) | CO purification rate (%) |
|              |                        |    |  | Oxidation                                                   |                          |                          |
| 18           | 24                     | 66 |  | 800°C<br>Oxidation<br>Reduction<br>after<br>oxidation       | 14.4                     | 30.0                     |
|              |                        |    |  | 900°C<br>Oxidation<br>Reduction<br>after<br>oxidation       | 36.0                     | 53.3                     |
|              |                        |    |  | 1000°C<br>Oxidation<br>Reduction<br>after<br>oxidation      | 76.8                     | 52.2                     |
|              |                        |    |  | 1100°C<br>Oxidation<br>Reduction<br>after<br>oxidation      | 54.3                     | 46.0                     |
|              |                        |    |  | 1000°C<br>Oxidation<br>Reduction<br>after<br>oxidation      | 0                        | 0                        |
|              |                        |    |  | 1100°C<br>Oxidation<br>Reduction<br>after<br>oxidation      | 58.2                     | 58.2                     |
|              |                        |    |  | 1000°C<br>Oxidation<br>Reduction<br>after<br>oxidation      | 0                        | 1                        |
|              |                        |    |  | 1100°C<br>Oxidation<br>Reduction<br>after<br>oxidation      | 62.0                     | 48.2                     |

Table 4

| Specimen No. | Chemical component (%) |      |     |                            | Fe-Ni-Cu additive element system alloys and purification rates |                          |
|--------------|------------------------|------|-----|----------------------------|----------------------------------------------------------------|--------------------------|
|              | Cu                     | Ni   | Fe  | Others                     | Oxidation/Reduction                                            | NO purification rate (%) |
|              |                        |      |     |                            | Oxidation                                                      |                          |
| 19           | 8.8                    | 30.4 | bal | C-1.0<br>Si-2.2<br>Co-21.4 | Not measured                                                   | 75.0                     |
| 20           | 9.8                    | 18.4 | bal | C-2.1<br>Si-2.3            | "                                                              | 72.1                     |
| 21           | 11.6                   | 39.8 | bal | C-1.6                      | "                                                              | 80.9                     |

Table 4-continued

| Specimen No. | Fe-Ni-Cu additive element system alloys and purification rates |      |     |                           | NO purification rate (%)<br>Oxidation/Reduction<br>Oxidation | Reduction<br>after<br>oxidation |
|--------------|----------------------------------------------------------------|------|-----|---------------------------|--------------------------------------------------------------|---------------------------------|
|              | Cu                                                             | Ni   | Fe  | Others                    |                                                              |                                 |
| 22           | 17.7                                                           | 47.6 | bal | Si-2.1<br>C-1.5<br>Si-1.6 | "                                                            | 72.0                            |
| 23           | 17.7                                                           | 32.0 | bal | Al-3.9                    | 3.7                                                          | 74.1                            |
| 24           | 18.9                                                           | 47.4 | bal | C-1.1<br>Si-1.6           | Not measured                                                 | 72.0                            |
| 25           | 27.9                                                           | 17.3 | bal | Si-4.3                    | 0                                                            | 75.3                            |
| 26           | 24.3                                                           | 39.1 | bal | Ce-4.1                    | 1.8                                                          | Not measured                    |
| 27           | 29.7                                                           | 3.7  | bal | Al-2.8                    | 2.8                                                          | 77.7                            |
| 28           | 30.1                                                           | 8.9  | bal | Si-3.1                    | 0                                                            | 70.4                            |

Table 5

| Specimen No. | Fe-Cu additive element system alloys and purification rate |     |         | NO purification rate (%)<br>Oxidation/Reduction<br>Oxidation | Reduction<br>after<br>oxidation |
|--------------|------------------------------------------------------------|-----|---------|--------------------------------------------------------------|---------------------------------|
|              | Cu                                                         | Fe  | Others  |                                                              |                                 |
| 29           | 9.4                                                        | bal | Co-36.5 | 21.4                                                         | 86.2                            |
| 30           | 19.0                                                       | bal | Si- 2.9 | 28.3                                                         | 56.5                            |
| 31           | 19.3                                                       | bal | Al- 3.0 | 1.2                                                          | 84.1                            |
| 32           | 20.8                                                       | bal | Ti- 3.2 | 2.4                                                          | 96.3                            |
| 33           | 28.9                                                       | bal | Co-33.0 | 4.0                                                          | 76.0                            |

Table 6

| Specimen No. | Ni-Cu additive element system alloys and purification rates |      |                    | Oxidation/Reduction                          | NO purification rate (%) |
|--------------|-------------------------------------------------------------|------|--------------------|----------------------------------------------|--------------------------|
|              | Cu                                                          | Ni   | Others             |                                              |                          |
| 34           | 4.1                                                         | 29.0 | Cr-20.5<br>Mo- 2.8 | Oxidation<br>Reduction<br>after<br>oxidation | 50.2<br>32.2             |

Reasons for restricting each component element in this system's alloy, which is a basis for the catalyst according to this invention, and its effect are presented below.

As for Cu, when this system's alloy has been oxidized and subsequently reduced to impart a catalyst effect, CuO\* is formed on the alloy surface, and CuO\* being diffused into FeO\* and NiO\* is presumed to play a significant role for catalytic effect.

CuO\* herein represents oxidized Cu, but since the state of achieving the optimum catalytic effect is unknown and content of oxygen can not be determined, representation is made by O\*.

Catalytic activity is deemed to become present when O\* in oxides is almost nil. FeO\* and NiO\* denote the same as in CuO\*.

When the surface of alloys subjected to oxidization treatment at high temperature was examined by utilizing X-ray diffraction to certify the above matters, compositions were proven as follows.

CuO\* - - - CuO  
FeO\* - - - Fe<sub>2</sub>O<sub>3</sub> (Hematite)  
NiO\* - - - NiO

Moreover, the following compositions were also clarified when the surface of the alloy was examined by

using X-ray diffraction after subjecting same to reduction treatment.

CuO\* - - - Cu (\* = 0)

FeO\* - - - Fe (\* = 0)

NiO\* - - - Ni (\* = 0)

However, it can not be concluded that all of them are in the same state as mentioned above.

The reason for restricting the Cu content is that when Cu exceeds 40% or becomes less than 0.1% by weight, diffusion of CuO\* into NiO\* and FeO\* becomes dense and coarse respectively, and either case adversely affects the catalytic effect. In case Cu is excessive, it separates and deposits in the alloy provided that it does not form a solid solution or intermetallic compound.

This problem is caused due to the presence of Fe as seen from the Fe-Cu binary state diagram given in FIG. 1, and deposited Cu does not have catalytic effect.

Intermetallic compounds are difficult to oxidize, and even if oxidized, those compounds do not form oxidized layers having catalytic effect. Therefore, although Cu is contained therein, it adversely affects the catalytic effect. The more this system's alloy contains solid solution Fe-Ni-Cu or Fe-Cu, the greater the catalytic effect becomes. Now, as for Ni and Fe, it is felt that Ni and Fe act to promote the catalytic effect rather than to provide the direct reduction effect to NO<sub>x</sub>, that is, a dispersed state of CuO\* is thereby made effective and the effect of adsorbing molecules such as CO and H<sub>2</sub> useful for reduction of NO is excellent.

Meanwhile, Ni is effective for expanding a solid solution limit of Cu into Fe, which can be presumed from the binary state diagram of Ni-Cu and Fe-Ni given in FIG. 1. Coexistence and independent existence of Ni and Fe are acceptable.

If additive elements satisfy the following conditions when added to this system's alloys of Fe-Ni-Cu, Fe-Cu or Ni-Cu, the catalytic effect will not be reduced much, that is;

1. Permeation into solid solution.
2. Non-production of intermetallic compound with Cu.
3. Non-deposition of Cu due to presence of additive elements.

Moreover, if additive elements less than 10% by weight satisfy the above conditions, the catalytic effect will be obtained. The less the degree of satisfying the conditions becomes, the lower the catalytic effect becomes, but as long as additive elements do not exceed 10% by weight, the catalytic effect will be substantially maintained.

Also, even if graphite is crystallized in the alloy structure by adding carbon or silicon, the catalytic effect will not be adversely effected. As for Co, it acts similarly to Cu as described previously and it is unnecessary to restrict the content of Co, but the upper limit is determined in relation to the coexistence with Fe and Ni. As for Cr, it does not considerably lower the catalytic effect and the content may widely be restricted. However, the content of Cr over 40% is undesirable from a standpoint of melting and subsequent workability.

In addition to the description as to component elements, microscopic photographs of casted and annealed structures of component elements given in Examples 1 through 6 are presented in FIGS. 3 through 8 in order to clarify the effect of each component. Annealed structures are those which are annealed by furnace cooling after heating at 1000°C. for 6 hours.

Then, actions of oxidized layers and reduced layers which are essential for obtaining optimum catalytic effect are described. Oxidized layers are formed by oxidizing in atmospheric conditions. Since thicknesses of oxidized layers vary with alloy compositions, surface condition, oxidizing temperature, and period of oxidizing time, treatment conditions can not be formulated, but desired thickness is obtainable by selecting conditions within temperatures ranging from 700° to 1100°C. and time periods ranging from 1/2 hour to 24 hours or temperatures ranging from 800 to 1300°C and time periods ranging from 3 to 24 hours.

The thickness of oxidized layers are required to be at least 10μ and a thickness above 10μ is unlimitedly permissible, to the extreme of up to the center portion of the alloys.

On the contrary, as the thickness becomes less than 10μ, the catalytic effect is remarkably deteriorated and at last becomes unobtainable if the temperature is above 700°C. This is considerably due to the effect of CuO\*, NiO\*, FeO\*, etc., against the catalytic activity as previously described in the compositions. Also, the oxidized layer with a thickness of at least 10μ is necessary to provide oxidized layers with corrugation and to increase the surface area as will be described later. As a result of examining composition variations of oxidized layers by using an X-ray micro-analyzer, the following matters became clear, that is enriched Fe and Cu layers are formed at the top surface, and moreover, the enriched Cu layer is placed close to the surface more than the enriched Fe layer. This tendency becomes further obvious by providing a reduction treatment and the enriched Cu layer exists at the very top surface.

An enriched Ni layer is also formed at the portion near the surface, but slightly lower than the enriched Fe and Cu layers, and after subsequent reduction treatment, in the same position as that of the enriched Fe layer or slightly close to the surface. The enriched Cu layer formed near the top surface exists independent from other additive elements. Co displays an enriched state similar to that of Cu.

In case the oxidized layer is thinner than 10μ, the enriched oxidized layer, as described above, can not be formed. On the other hand, as the oxidized layer becomes thicker, the above tendency becomes considerably more, that is, Cu enriches in the surface and diffuses into Ni and Fe. This is an advantageous condition for catalytic effect. In Examples 1-6, since the thickness of all oxidized layers were made in 0.5 - 1.0mm,

the above condition was satisfied. As a result of observing oxidized layer surfaces by a scanning-type microscope, it became clearer that the oxidized layer surfaces were corrugated and porous, that this tendency became extreme when the oxidized layer thickness was less than 10μ, and further, that this tendency became obvious when the oxidized layer was subjected to a subsequent reduction treatment.

Thus, an oxidized layer thinner than 10μ apparently lowers its catalytic effect, as seen from the above surface observation results. This tendency is shown in FIGS. 9 and 10. FIG. 9 shows the surface when the oxidized layer is insufficiently formed and corrugation and porosity are not seen therein, but are apparent in FIG. 8 which shows the state of a sufficiently oxidized layer.

As described in the Examples, the reduction treatment of an oxidized layer is the processing in hydrogen gas and the treatment condition is determined within the treatment period of time ranging from 1/2 - 24 hours in accordance with the state of the subject oxidized layer, and at least, partial treatment is acceptable.

Thereafter, the test results on catalytic effects by catalysts according to the present invention are presented.

#### TEST EXAMPLE 1

The purification rate as to NO was measured under the following conditions in order to certify the effect of each catalyst obtained in the embodying Examples 1-6.

| 35                        |  | (1) Test conditions                                          |  |
|---------------------------|--|--------------------------------------------------------------|--|
| Devices employed:         |  | NO purification analyzer using a flow-type mini-reactor      |  |
| Test gas:                 |  | NO measuring meter.                                          |  |
| Gas flow rate:            |  | CO 1%                                                        |  |
| Amount of catalyst:       |  | NO 1000 ppm                                                  |  |
| Type of catalyst:         |  | O <sub>2</sub> 0.24%                                         |  |
| S.V. (Space Velocity):    |  | N <sub>2</sub> the rest                                      |  |
|                           |  | 2.75 liter/minute                                            |  |
|                           |  | 10ml in cuttings or bent sheet                               |  |
|                           |  | Catalysts obtained in embodying examples                     |  |
|                           |  | Approx. 16500 v/v, hr <sup>-1</sup>                          |  |
|                           |  | V <sub>p</sub> : Apparent volume of a charged catalyst layer |  |
|                           |  | V: Gas flow rate                                             |  |
| Catalyst bed temperature: |  | Approx. 400°C.                                               |  |
| Catalyst surface area:    |  | Apparent area of approx.                                     |  |
|                           |  | 100 ~ 1000cm <sup>2</sup> dependent on shapes                |  |

#### 2. Results

The results are as given in Tables 1 through 6. Each result shows an excellent NO purification rate. Certain catalysts do not achieve sufficient purification ability with their oxidized layers only, but it has been known that the effect can be improved by providing same with reduction treatment. As a result of testing with alloy systems other than this system's alloy under the same conditions, neither one demonstrated a sufficient NO purification rate.

The catalysts according to the present invention also act effectively as an oxidization catalyst for hydrocarbon (HC) and carbon monoxide (CO) if an oxidization atmosphere is available.

## TEST EXAMPLE 2

The test was made under the following conditions by using the same analyzing devices as in Test Example 1.

## (1) Test Conditions

CO measuring meter was used.  
Test gas: CO 1%  
NO 2000 ppm  
O<sub>2</sub> 0.25%  
N<sub>2</sub> the rest

## TEST EXAMPLE 3

This test proves that the catalysts according to this invention are effective for purifying harmful NO components contained in internal combustion engine exhaust gas.

The catalyst was made by machining this system's alloy with various components, as given in Table 7, to produce cuttings by forming an oxidized layer, by reducing, and then stuffing into the catalyst converter for purifying internal combustion engine exhaust gas.

| (1) Test conditions                          |                                                                                                                                     |
|----------------------------------------------|-------------------------------------------------------------------------------------------------------------------------------------|
| Internal combustion engine:                  | 1900cc four cylinder reciprocal gasoline engine                                                                                     |
| Installation location of catalyst converter: | Just behind the exhaust manifold and approximately 40cm back from the cylinder head                                                 |
| Shape of catalyst converter:                 | Cylindrical type with 70mm diameter and 300mm length.                                                                               |
| Type of catalyst:                            | Capacity 1.2 lit.<br>Catalysts with compositions given in Table 7.<br>Stuffed compactly.<br>Weight: Approx. 2.0kg                   |
| Engine operation: Condition:                 | Apparent surface area: Approx. 20000 cm <sup>2</sup><br>Steady bench test operation<br>A 2700 rpm 2.2kg - m<br>B 2500 rpm 1.2kg - m |
| Catalyst bed temperature:                    | A 660°C.<br>B 630°C.                                                                                                                |
| S.V.:                                        | A 40,000 V/V <sub>p</sub> hr <sup>-1</sup><br>B 27,000 V/V <sub>p</sub> hr <sup>-1</sup>                                            |

|                           |                                                                                                                              |
|---------------------------|------------------------------------------------------------------------------------------------------------------------------|
| Gas flow rate:            | 2.5 l/minute                                                                                                                 |
| Amount of catalyst:       | 5ml                                                                                                                          |
| Type of catalyst:         | Ni-24% Cu catalyst in a bent sheet with 50 cm <sup>2</sup> of apparent surface area 30,000 v/v <sub>p</sub> hr <sup>-1</sup> |
| S.V.:                     | 300 - 700°C.                                                                                                                 |
| Catalyst bed temperature: |                                                                                                                              |

Measurement was made by an exhaust gas analyzing meter.

## 2. Results

35 NO and CO were purified approximately 40 - 100% and 11% respectively, as shown in Table 7. As a result of testing with alloys other than this system's alloy, both achieved a slight purification rate.

Table 7

| Specimen | Alloy component (%) |      |     |                               | Engine operating condition | NO purification rate | CO purification rate |
|----------|---------------------|------|-----|-------------------------------|----------------------------|----------------------|----------------------|
|          | No.                 | Cu   | Ni  | Fe                            |                            |                      |                      |
| 35       | 9.4                 | 45.0 | bal |                               | A                          | 58.3                 | 10.7                 |
| 36       | 9.0                 | 43.3 | bal | Cr- 3.7                       | A                          | 98.0                 | 5.0                  |
| 37       | 9.2                 | 39.5 | bal | Co- 1.3                       | B                          | 55.5                 | 9.9                  |
| 38       | 8.9                 | 41.7 | bal | Co-15.7                       | A                          | 94.4                 | 4.6                  |
| 39       | 8.8                 | 42.6 | bal | Co- 5.3<br>Cr- 4.1<br>Ce- 2.5 | B                          | 40.5                 | 8.3                  |
|          |                     |      |     |                               | A                          | 89.9                 | 4.7                  |
|          |                     |      |     |                               | B                          | 49.7                 | 9.1                  |
|          |                     |      |     |                               | A                          | 92.3                 | 5.0                  |
|          |                     |      |     |                               | B                          | 45.2                 | 8.9                  |
|          |                     |      |     |                               | A                          | 88.3                 | 4.4                  |

## Note:

Average exhaust gas composition under operating condition A  
NO-2400 ppm CO-2.2% HC-110 ppm  
Average exhaust gas composition under operating condition B  
NO-600 ppm CO-4.5% HC-160 ppm

## 2. Results

Both NO and CO were remarkably purified from the low temperature side as illustrated in FIG. 2. The term "Oxidization" given in FIG. 2 denotes that an oxidized layer formed by treating in atmosphere at 900°C. for 12 hours was present and the term "Reduction after oxidation" denotes that it was subsequently subjected to hydrogen gas reduction at 800°C. for 2 hours.

As seen from the evaluations based on the above test examples, this system's alloy achieves an outstanding effect as reduction oxidation catalysts. Also as proven by embodying examples and test examples, the alloy is obtainable at low cost due to extensive selection range of alloys. Moreover, the alloy is a highly strong and excellent in plasticity, workability and castability as well as heat resistance and corrosion resistance. There-

**11**

fore, it can advantageously be formed into cuttings, sheets, pipes, etc. according to application.

What is claimed is:

1. An exhaust gas purifying catalyst comprising an alloy consisting essentially of 0.1-40% Cu and the balance of at least one of the group consisting of Ni, Fe, and a combination of Ni and Fe by weight as fundamental components, and including a surface formed by first oxidizing the alloy by heating at 700°C. - 1100°C. in an oxidizing atmosphere for  $\frac{1}{2}$  to 24 hours to provide an oxidized layer at least  $10\mu$  in thickness, and thereafter reducing the oxidized layer in a reducing atmosphere at approximately 800°C. for about 2 hours.

**12**

2. An exhaust gas purifying catalyst according to claim 1 including 40% or less of at least one of the group consisting of Co and Cr.

3. A process of producing a catalyst for purifying exhaust gas which comprises shaping an alloy as desired containing 0.1 - 40% of Cu and the balance of at least one of Ni and Fe as fundamental components and forming an oxidized layer of more than  $10\mu$  in thickness on the surface of said shaped alloy by heating same at 800°- 1300°C. in an oxidization atmosphere for 3 - 24 hours, and thereafter reducing the oxidizing layer by heating same in a reducing atmosphere at approximately 800°C. for about 2 hours.

\* \* \* \* \*

15

20

25

30

35

40

45

50

55

60

65